

# UNITED STATES PATENT OFFICE.

JOHN C. SELLARS, OF BIRKENHEAD, COUNTY OF CHESTER, ENGLAND.

## COMPOSITION FOR MOLDS AND COMPOSITION-MOLD FOR FORMING CONCRETE.

SPECIFICATION forming part of Letters Patent No. 244,321, dated July 12, 1881.

Application filed May 31, 1881. (No specimens.) Patented in England April 9, 1877.

*To all whom it may concern:*

Be it known that I, JOHN CARRINGTON SELLARS, of Birkenhead, in the county of Chester, England, have invented a new and useful 5 Composition for Molds and Composition-Mold for Forming Concrete, Artificial Stone, Cement, and like Substances, (for which I have obtained a patent in Great Britain, No. 1,379, bearing date April 9, 1877,) of which the following is 10 a specification.

Concrete, artificial stone, cement, and like substances have not hitherto been made available for ornamental purposes generally, or where great diversity of form or shape has 15 been requisite, on account of the difficulty of giving the desired outline to the said concrete, artificial stone, cement, and like substances.

Now the object of my invention is to provide a composition of matter specially adapted 20 for the formation of molds in which to pour or fill concrete, artificial stone, cement, or like substances, in a liquid or semi-liquid condition, so as to obtain a casting of sharp, clear, and well-defined outline, and of smooth, neat, and 25 finished appearance.

The great obstacle to making castings of concrete or artificial stone has been the facility with which such concrete or stone has adhered to the surface of the mold, rendering 30 the removal of the casting from the said mold difficult, and a disfigured and rough article, quite unfit for use from an artistic point of view, has been produced.

By my invention perfect concrete or like 35 castings of any form or design obtainable in metal can be easily formed, and the invention is specially applicable to the manufacture of letters and objects decorated with foliage and other complicated designs.

In carrying my invention into practice the 40 molds in which the concrete, artificial stone, cement, or like substances are cast are formed or made of the following ingredients combined in the proportions stated: sand, charcoal, or finely-divided material, one hundred parts, by 45 weight; paraffine or similar wax-like substance unacted upon by alkaline matter, from six to eleven parts, by weight.

Molds made with ninety-three parts, by weight, of sand and seven, by weight, of paraffine answer well.

The impressions are formed in the composition by means of patterns, as is usual in making molds for metal casting.

To insure that the casting shall be smooth 55 and well finished, steam or hot air is passed over the surface of the composition-mold before the concrete or the like is poured or filled in.

What I claim, and desire to secure by Letters Patent of the United States, is—

1. A composition to be used in the formation of molds for shaping concrete and like plastic material, the same consisting of a lubricating binding material which is not affected by alkalies—such as paraffine—and a finely-divided body material—such as sand or charcoal—substantially as and for the purpose specified.

2. A composition-mold for shaping concrete and like plastic material, composed of paraffine and sand or charcoal, substantially in the proportions and for the purpose specified.

JNO. C. SELLARS.

Witnesses:

J. JOHNSON,  
J. RICHMAN.